

# UNITED STATES PATENT OFFICE.

PAUL B. HERSMAN, OF MILWAUKEE, WISCONSIN, ASSIGNOR, BY MESNE ASSIGNMENTS,  
TO WILLIAM F. JOBBINS, INCORPORATED, OF AURORA, ILLINOIS, A CORPORATION  
OF ILLINOIS.

## METHOD OF PROCESSING ALUMINUM SKIMMINGS, SCREENINGS, SLAGS, OR ANALOGOUS MATERIALS.

1,229,611.

Specification of Letters Patent. Patented June 12, 1917.

No Drawing.

Application filed November 14, 1912. Serial No. 731,347.

To all whom it may concern:

Be it known that I, PAUL R. HERSMAN, a subject of the Emperor of Austria, residing at Milwaukee, in the county of Milwaukee and State of Wisconsin, have invented new and useful Improvements in Methods of Processing Aluminum Skimmings, Screenings, Slags, or Analogous Materials, of which the following is a full, clear, concise, and exact description.

This invention relates to a method of utilizing aluminum skimmings, screenings, slags or analogous materials in such a way as to produce certain valuable and useful products. In carrying out my invention I prefer the following procedure:

The skimmings are first separated by suitable means from the large pieces of metal occurring with them. The residual skimmings consist of aluminum, aluminum alloys and carbide, nitrid, oxid, carbonate and other compounds of aluminum, small quantities of iron and copper and their compounds, carbon and other impurities. Since the aluminum and its alloys, left in this residual material, are present in a finely divided condition in which they cannot readily be separated from the non-metallic constituents of the material, the material is best now subjected to the following process which effects a melting together of the fine metal into larger fragments and at the same time not only avoids the decomposition of the nitrid originally present in the material, but usually appreciably increases the nitrid content of the non-metallic portion of the skimmings, etc. The skimmings, etc., from which the larger fragments of metal have been removed, are intimately mixed with a hydrocarbon such as tar, asphaltum, petroleum oil, resin oil, or like material, the operation preferably being carried out at such temperature that the hydrocarbon used is freely fluid in order that the individual particles of the skimmings may be coated as completely as possible with the hydrocarbon. It will be understood that the hydrocarbons when added to the skimmings may be in any form so long as they are of such nature that they will become fluid and will therefore become thoroughly mixed with, and be able to act as a coating for, the skimmings before the mixture attains the temperature at which

the step of exposure to the air is to take place. The mass is then heated in a closed retort until the mixture has been brought to approximately 1,200 degrees centigrade; it is then quickly exposed to the air, whereupon an automatic heating accompanied by a considerable rise of temperature takes place, during the progress of which the desired reaction is completed. Magnetic iron and whatever aluminum has been fused into large particles during the process may then be separated by suitable means. The residue, now practically free from metallic aluminum or its alloys and containing usually an increased amount of available nitrogen, is treated with boiling water, preferably in the presence of lime, or with other alkaline agents to release from the mass its available nitrogen in the form of ammonia, which ammonia may then be collected in water and concentrated in order to become a commercial product, or if preferred, it may be transformed into salts of ammonia by well known means. The remaining material may be treated for the recovery from it of aluminum sulfate or of other compounds of aluminum and compounds of copper which possess commercial value.

While the procedure described constitutes the preferred process, it is understood that various changes may be made in it without departing from the spirit of the invention. Thus skimmings and analogous materials which have been finely ground and then exposed to moisture and air contain very little free metal and therefore it will in some cases be preferable to omit the treatment with a hydrocarbon and heat and to proceed at once with the release of the original nitrogen content of the material and the regaining of its luminous content and the copper compounds, as above described. Other changes, also, such as making the various processes continuous, as will readily suggest themselves to those skilled in the art may be made without departing from the spirit of the invention.

Having thus described my invention, what I claim as new and desire to secure by Letters Patent is—

1. A method of utilizing aluminum skimmings, screenings, slags and the like which consists in mixing the same with a reducing

agent, heating the mixture in a closed retort without access of nitrogen to a temperature at which aluminum nitrid is formed and then exposing it to an atmosphere containing nitrogen.

2. A method of utilizing aluminum skimmings, screenings, slags and the like which consists in mixing the same with a reducing agent, heating the mixture in a closed 10 retort without access of air to a temperature at which aluminum nitrid is formed and then exposing it to the air.
3. A method of utilizing aluminum skimmings, screenings, slags and the like which 15 consists in mixing the same with a reducing agent, heating the mixture without access of nitrogen to a temperature of approximately 1200° centigrade, and then exposing it to an atmosphere containing nitrogen.
4. A method of utilizing aluminum skimmings, screenings, slags and the like which 20 consists in mixing the same with a liquid hydrocarbon, heating the mixture in a closed retort without access of nitrogen to a temperature at which nitrid of aluminum is 25 formed and then exposing it to an atmosphere containing nitrogen.
5. A method of utilizing aluminum skimmings, screenings, slags and the like which 30 consists in mixing the same with a reducing agent, heating the mixture in a closed retort without access of air to a temperature such

that when the same is exposed to the air an automatic heating action takes place and then exposing the mixture to the air.

35

6. The method of processing aluminum skimmings, screenings, slags or analogous materials, which consists in mixing the same with a hydrocarbon in liquid form, heating the mixture with access of minimal quantities of air, and subsequently exposing the mass to excess of air, the heating having been carried to such point that a considerable rise of temperature results when the mass is so exposed to the air.

45

7. The method of utilizing aluminum skimmings, screenings, slags or analogous materials, which consists in mixing the same with a hydrocarbon in liquid form, heating the mixture in a closed retort, subsequently exposing the mass to the air, the heating in the closed retort having been carried to such a point that automatic heating results when the mass is exposed to the air, and then finally separating from the mass the larger 50 particles of metal formed during the process.

50

In witness whereof, I have hereunto subscribed my name in the presence of two witnesses.

PAUL R. HERSMAN.

Witnesses:

JAMES A. LAURIE,  
JNO. R. McGREGOR.